# EUROPEAN PATENT SPECIFICATION

(11) **EP 1 085 105 B1**
(45) Date of publication and mention of the grant of the patent: **28.06.2006**
(21) Application number: 00118990.1
(22) Date of filing: 01.09.2000
(51) Int. Cl.: C22C 38/60, C22C 38/40, C22C 38/28, C22C 38/18, C22C 19/05, C22C 27/06

(54) **Free cutting alloy**
Automatenlegierung
Alliage de décolletage

(30) Priority: 03.09.1999 JP 25090299; 14.03.2000 JP 2000070257; 21.07.2000 JP 2000221433; 22.08.2000 JP 2000251602; 22.08.2000 JP 2000251626
(43) Date of publication of application: 21.03.2001
(62) Divisional of application: 04004043.8
(73) Proprietor: Tohoku Technoarch Co., Ltd., Sendai-shi, Miyagi 980-0845 (JP); Japan Industrial Technology Association, Tokyo 105-0001 (JP); Oikawa, Katsunari, Shibata-gun, Miyagi (JP); Tohoku Tokushuko Kabushiki Kaisha, Shibata-gun, Miyagi (JP); Daido Tokushuko Kabushiki Kaisha, Naka-ku Nagoya-shi Aichi-ken (JP); Ishida, Kiyohito, Sendai-shi, Miyagi-ken (JP)
(72) Inventor: Ishida, Kiyohito, Sendai-shi, Miyagi (JP); Oikawa, Katsunari, Shibata-gun, Miyagi (JP); Ebata, Takashi, c/o Tohoku Tokushuko K.K., Shibata-gun, Miyagi (JP); Inoguchi, Takayuki, Tokai-shi, Aichi (JP); Shimizu, Tetsuya, Nagoya-shi, Aichi (JP); Okabe, Michio, Chita-shi, Aichi (JP)
(74) Representative: ter Meer, Nicolaus

(56) References cited:
- EP-A- 0 767 247
- EP-A- 0 903 418
- GB-A- 1 519 313
- US-A- 4 705 581
- PATENT ABSTRACTS OF JAPAN vol. 1999, no. 13, 30 November 1999 (1999-11-30) -& JP 11 229082 A (SUMITOMO METAL IND LTD), 24 August 1999 (1999-08-24)
- R.KIESSLING ET AL: "Non-metallic inclusions in steel" 1978 , THE INSTITUTE OF MATERIALS , LONDON, GB XP002155733 * page 138, line 10 - line 17 * * page 139, line 21 - line 22 * * page 144, paragraph K14 - page 145, line 15 *
- PATENT ABSTRACTS OF JAPAN vol. 1999, no. 13, 30 November 1999 (1999-11-30) -& JP 11 229032 A (SUMITOMO METAL IND LTD), 24 August 1999 (1999-08-24)
- PATENT ABSTRACTS OF JAPAN vol. 2000, no. 01, 31 January 2000 (2000-01-31) -& JP 11 293390 A (SUMITOMO METAL IND LTD), 26 October 1999 (1999-10-26)
- PATENT ABSTRACTS OF JAPAN vol. 1998, no. 10, 31 August 1998 (1998-08-31) -& JP 10 130794 A (DAIDO STEEL CO LTD), 19 May 1998 (1998-05-19)
- PATENT ABSTRACTS OF JAPAN vol. 012, no. 333 (C-526), 8 September 1988 (1988-09-08) -& JP 63 093843 A (DAIDO STEEL CO LTD), 25 April 1988 (1988-04-25)
- PATENT ABSTRACTS OF JAPAN vol. 014, no. 439 (C-0761), 19 September 1990 (1990-09-19) -& JP 02 170948 A (DAIDO STEEL CO LTD), 2 July 1990 (1990-07-02)
- PATENT ABSTRACTS OF JAPAN vol. 1999, no. 10, 31 August 1999 (1999-08-31) -& JP 11 140597 A (DAIDO STEEL CO LTD), 25 May 1999 (1999-05-25) & US 6 033 625 A (T. NAGASHIMA ET AL) 7 March 2000 (2000-03-07)
- PATENT ABSTRACTS OF JAPAN vol. 009, no. 324 (C-320), 19 December 1985 (1985-12-19) -& JP 60 155653 A (HITACHI SEISAKUSHO KK), 15 August 1985 (1985-08-15)

## Description

The present invention relates to free cutting alloy excellent in machinability.

Alloy has widespread applications because of a variety of characteristics thereof. A free cutting alloy excellent in machinability is, in a case, selected for improvement of productivity. In order to improve machinability, for example, free cutting alloy containing an element improving machinability such as S, Pb, Se or Bi (hereinafter referred to as machinability-improving element) is widely used. Especially in a case where machinability is particularly required because of precise finishing in machining or for other reasons, not only is a content of such a machinability-improving element increased in an alloy, but the elements are also added to an alloy in combination.

While S, which has widely been used for improvement of machinability, is in many cases added in the form of MnS, addition thereof in an alloy in a large content causes for degrading corrosion resistivity, hot workability and cold workability of the alloy. Moreover, when the alloy is exposed to the air, a sulfur component included in the alloy is released into the air in the form of a sulfur containing gas, which causes sulfur contamination in peripheral areas of parts with ease. Therefore, there arises a necessity of suppressing release of sulfur containing gas (hereinafter referred to as improvement on out-gas resistivity). Elements such as S, Se and Te, however, deteriorate magnetic properties to a great extent in an electromagnetic stainless steel and the like.

Therefore, various proposals have been made: a Mn content is limited, a Cr content in sulfide is increased or in a case where S is contained, Ti is added in combination with S in order to disperse sulfide in the shape of a sphere (for example, see JP-A-98-46292 or JP-A-81-16653). To increase a Cr content in sulfide, however, tends to greatly decrease in machinability and hot workability and therefore, such a alloy has been restricted on its application in many cases.

Specific steels having improved machinability and/or fatigue resistance and wear resistance and/or workability in general have been disclosed in JP 11229032, EP 0 903 418, JP 11229082, and EP 0 767 247.

It is accordingly an object of the present invention is to provide free cutting alloy excellent in machinability, showing outstanding characteristics as an alloy such as corrosion resistivity, hot workability and cold workability or specific magnetic characteristics, which are comparable to those of conventional alloys.

### Summary of the Invention

In order to achieve the above described object, a free cutting alloy of the present invention is characterized by the free cutting alloy of claim 1. "(Ti,Zr)" means one or two of Ti and Zr.

Machinability of an alloy can be improved by forming the above described (Ti, Zr) based compound in a matrix metal phase of the alloy. Furthermore, by forming this compound in the alloy, formation of compounds such as MnS and (Mn,Cr)S, easy to reduce corrosion resistivity and hot workability of the alloy, can be prevented or suppressed, thereby enabling corrosion resistivity, hot workability and cold workability to be retained at good levels. That is, according to the present invention, a free cutting alloy excellent in machinability can be realized without any degradation in useful characteristics as an alloy such as hardness, corrosion resistivity, hot workability, cold workability and specific magnetic characteristics.

Further, a (Ti,Zr) based compound formed in a free cutting alloy of the present invention is dispersed in the alloy structure. Machinability of an alloy can be further increased especially by dispersing the compound in an alloy structure. In order to increase the effect, a particle size of the (Ti,Zr) based compound as observed in the structure of a polished section of the alloy is preferably, for example, approximately in the range of 0.1 to 30 µm on the average and further, an area ratio of the compound in the structure is preferably in the range of 1 to 20 %, wherein the particle size is defined by the maximum distance between two parallel lines circumscribing a particle in observation when parallel lines are drawn intersecting on a region including the particle in observation while changing a direction of the parallel lines.

The above described (Ti,Zr) based alloy can include at least a compound expressed in a composition formula (Ti,Zr)₄(S,Se,Te)₂C₂ (hereinafter also referred to as carbo-sulfide/selenide), wherein one or more of Ti and Zr may be included in the compound and one or more of S, Se and Te may be included in the compound. By forming a compound in the form of the above described composition formula, not only can machinability of an alloy be improved, but corrosion resistivity is also improved.

It should be appreciated that identification of a (Ti,Zr) based compound in an alloy can be performed by X-ray diffraction (for example, a diffractometer method), an electron probe microanalysis method (EPMA) and the like technique. For example, the presence or absence of the compound of (Ti,Zr)₄(S,Se,Te)₂C₂ can be confirmed according to whether or not a peak corresponding to the compound appear in a diffraction chart measured by an X-ray diffractometer. Further, a region in the alloy structure in which the compound is formed can also be specified by comparison between two-dimensional mapping results on characteristic X-ray intensities of Ti, Zr, S, Se or C obtained from a surface analysis by EPMA conducted on a section structure of the alloy.

### Brief Description of the Drawings

Fig. 1 is a graph showing an X-ray diffraction chart of an inventive steel specimen No. 5 in experiment of Example 1;
Fig. 2 is a graph showing an example of Schaeffler diagram;
Fig. 3 is an optical microphotograph of the first selection inventive steel specimen No.5 in Example 1;
Fig. 4 is a graph showing dependencies of solubility products on temperature of components of TiO, TiN, Ti₄C₂S₂, TiC, TiS and CrS in γ-Fe;

### Preferred Embodiments of the Invention

The present invention, to be concrete, is applied on an alloy constituted as stainless steel. In this case, in order to form a (Ti,Zr based compound without any degradation in characteristics as stainless steel, such an alloy contains one or more of Ti and Zr such that W_{Ti} + 0.52 W_{Zr} = 0.03 to 3.5 mass %, wherein W_{Ti} and W_{Zr} denote respective contents in mass % of Ti and Zr; and one or more of S and Se in the respective ranges of 0.01 to 1.0 mass % for S and 0.01 to 0.8 mass % for Se.

The reason why the elements and contents thereof are selected as follows:

### (1) The Ti and Zr content being defined such that W_{Ti} + 0.52 W_{Zr} = 0.03 to 3.5 mass %, wherein W_{Ti} and W_{Zr} denote respective contents in mass % of Ti and Zr

Ti and Zr are indispensable elements for forming a (Ti,Zr) based compound playing a central role in exerting the effect of improving machinability of a free cutting alloy of the present invention. When a value of W_{Ti} + 0.52 W_{Zr} is lower than 0.03 mass %, the (Ti,Zr) based compound is insufficiently formed in amount, thereby disabling the effect of improving machinability to be satisfactorily exerted. On the other hand, when in excess of the value, machinability is reduced on the contrary. For this reason, the value of W_{Ti} + 0.52 W_{Zr} is required to be suppressed to 3.5 mass % or lower. The above effect exerted when Ti and Zr are added into an alloy is determined by the sum of the numbers of atoms (or the sum of the numbers of values in mol), regardless of kinds of metals, Ti or Zr. Since a ratio between atomic weights is almost 1 : 0.52, Ti of a smaller atomic weight exerts a larger effect with a smaller mass. Thus, a value of W_{Ti} + 0.52 W_{Zr} is said to be compositional parameter reflects the sum of the numbers of atoms of Zr and Ti included in an alloy.

### (2) One or more of S and Se in the respective ranges of 0.01 to 1 mass % for S and 0.01 to 0.8 mass % for Se

S and Se are elements for useful in improving machinability. By adding S and Se into an alloy, in an alloy structure, formed is a compound useful for improving machinability (for example, a (Ti,Zr) based compound expressed in the form of a composition formula (Ti,Zr)₄(S,Se)₂C₂). Therefore, contents of S and Se are specified 0.01 mass % as the lower limit. When the contents are excessively large, there arises a chance to cause a problem of deteriorating hot workability and therefore, there have to be the upper limits: The S content is set to 1 mass % and the Se content is set to 0.8 mass % as the respective upper limits. Further, S and Se are both desirably added into an alloy in a necessary and sufficient amount in order to form a compound improving machinability of the alloy, such as the above described (Ti,Zr) based compound. An excessive addition of S results in deterioration of the out-gas resistivity.

A free cutting alloy constituted as stainless steel of the present invention is to be more detailed, ferrite containing stainless steel (hereinafter referred to as a first selection invention), wherein a composition of the free cutting alloy of the present invention is as follows:
The free cutting alloy contains: 2 mass % or lower, including zero, Ni; 12 to 35 mass % Cr; and 0.005 to 0.4 mass % C.

The reason why the constituting elements and contents thereof in the first selection invention constituted as ferrite containing stainless steel are determined is as follows:

### (3) 0.005 to 0.4 mass % C

C is an important element forming a compound improving machinability. When a content thereof is lower than 0.005 mass %, however, an effect exerting sufficient machinability can not be imparted to the alloy, while when in excess of 0.4 mass %, much of a single carbide not effective for improving machinability is formed. Addition of C is preferably set in the range of 0.01 to 0.1 mass %, wherein it is preferable that addition of C is adjusted so properly that the effect of imparting machinability on the alloy is optimized depending on an amount of a constituting element of a compound improving machinability such as a (Ti,Zr) based compound.

### (4) 2 mass % or lower, including zero Ni

Ni can be added according to a necessity since the element is effective for improving corrosion resistivity, particularly in an environment of a reducing acid. Excessive addition, however, not only reduce stability of a ferrite phase, but also causes cost-up and therefore, a content thereof has the upper limit of 2 mass %, wherein a case of no addition of Ni may be included.

### (5) 12 to 35 mass % Cr

Cr is an indispensable element for ensure corrosion resistivity and is added in the range of 12 mass % or higher. On the other hand, excessive addition is not only harmful to hot workability but also causes reduction in toughness and therefore the upper limit is set to 35 mass %.

Further, free cutting alloys of the first selection invention of the present invention constituted as ferrite containing stainless steel can contain: 2 mass % or lower, including zero Si; 2 mass % or lower, including zero Mn; 2 mass % or lower, including zero Cu; and 2 mass % or lower, including zero Co. In addition, the free cutting alloys can further contain one or more of Mo and W in the respective ranges of 0.1 to 4 mass % for Mo and 0.1 to 3 mass % for W.

Description will be given of the reason why the elements and contents thereof are defined as follows:

### (6) 2 mass % or lower, including zero Si

Si is added as a deoxidizing agent for steel. That Si is added in excess, however, is unfavorable because not only cold workability is deteriorated, but formation of δ ferrite increases in amount, thereby degrading hot workability of steel. Consequently, a Si content has the upper limit of 2 mass %. In a case where cold workability is particularly regarded as important, the Si content is preferably set 0.5 mass % or lower, including zero.

### (7) 2 mass % or lower, including zero Mn

Mn acts an deoxidizing agent for steel. In addition, since a compound useful for increase in machinability in co-existence with S or Se, there arises a necessity of addition when machinability is highly thought of. On the other hand, since MnS especially deteriorates corrosion resistivity, affects cold workability adversely. Therefore a Mn content has the upper limit of 2 mass %. Especially when corrosion resistivity and cold workability are regarded as important, a Mn content is desirably limited to 0.4 mass % or lower, including zero.

### (8) 2 mass % or lower, including zero Cu

Cu can be added according to a necessity since the element is effective for improving corrosion resistivity, particularly in an environment of a reducing acid. It is preferable to contain 0.3 mass % or higher in order to obtain a more conspicuous effect of the kind. When in excess, hot workability decreases whereby it is preferable for a Cu content to be set 2 mass % or lower, including zero. Especially when hot workability is regarded as important, it is more desirably to suppress the Cu content to 0.5 mass % or lower, including zero.

### (9) 2 mass % or lower, including zero Co

Co is an element effective for improving corrosion resistivity, particularly in an environment of a reducing acid. To contain Co in content equal to 0.3 mass % or higher is preferable in order to obtain more of conspicuousness in the effects. When added in excess, however, not only does hot workability decrease, but a raw material cost increases, and therefore, it is preferable to set a content of Co in the range of 2 mass % or lower, including zero. Especially when hot workability and decrease in raw material cost are regarded as important, a content of Co is more desirably suppressed to 0.5 mass % or lower, including zero.

### (10) One or more of Mo and W in the respective ranges of 0.1 to 4 mass % for Mo and 0.1 to 3 mass % for W

Since Mo and W can further increase corrosion resistivity and a strength, the elements may be added according to a necessity. The lower limits are both 0.1 %, where the effects thereof become clearly recognized. On the other hand, when added in excess, hot workability is deteriorated. Therefore, the upper limits of Mo and W are set 4 mass % and 3 mass %, respectively.

In the ferrite containing stainless steel, described above, contents of other elements are as follows: the stainless steels can contain: 0.05 mass % or lower P; and 0.03 mass % O; and 0.05 mass % or lower N. Moreover, the stainless steels can further contain one or more of Te, Bi and Pb in the respective ranges of 0.005 to 0.1 mass % for Te; 0.01 to 0.2 mass % for Bi; and 0.01 to 0.3 mass % for Pb. Description will be given of the reason why the elements and contents thereof are defined as follows:

### (11) 0.05 mass % or lower, including zero P

P is segregated at grain boundaries and not only increases intergranular corrosion sensibility but also sometimes reduces toughness. Therefore, a P content is preferably set as low as possible and to 0.05 mass % or lower, including zero. Although the P content is more desirably set to 0.03 mass % or lower, including zero, reduction in content more than necessary has a chance to be reflected on increased production cost.

### (12) 0.03 mass % or lower, including zero O

O combines with Ti or Zr both of which are constituting elements of a compound useful for improving machinability and forms oxides not useful for improving machinability. Therefore, an O content should be suppressed as low as possible and is set to 0.03 mass % as the upper limit. The O content is desirably set to 0.01 mass % or lower if allowable in consideration of increase in production cost.

### (13) 0.05 mass % or lower, including zero N

N combines with Ti or Zr both of which are constituting elements of a compound useful for improving machinability and forms nitrides not useful for improving machinability. Therefore, a N content should be suppressed as low as possible and is set to 0.05 mass % as the upper limit. The N content is desirably set to 0.03 mass % or lower, including zero and more desirably to 0.01 mass %, if allowable in consideration of increase in production cost.

### (14) One or more of Te, Bi and Pb in the respective ranges of 0.005 to 0.1 mass % for Te; 0.01 to 0.2 mass % for Bi; and 0.01 to 0.3 mass % for Pb

Since Te, Bi and Pb can further improve machinability, the elements may add if necessary. The lower limits thereof at which the respective effects are exerted to clearness are as follows: 0.005 mass % Te; 0.01 mass % Bi and 0.01 mass % Pb, respectively. On the other hand, since excessive addition reduces hot workability, the upper limits are set as follows: 0.1 mass % Te; 0.2 mass % Bi; and 0.3 mass % Pb.

Furthermore, the free cutting alloy of the present invention constituted as stainless steel can contain one or more selected from the group consisting of Ca, Mg, B and REM (one or more of metal elements classified as Group 3A in the periodic table of elements) in the range of 0.0005 to 0.01 mass % for one element or as a total content in a case of two or more elements. The elements are useful for improving hot workability of steel. The effect of improving hot workability obtainable by addition of the elements is more conspicuously exerted in the range of 0.0005 mass % or higher for one element or as a total content of more than one elements combined. On the other hand, when the elements are added in excess, the effect is saturated and hot workability is then reduced on the contrary. Therefore, the content of a single element or total content of the elements combined is set to 0.01 mass % as the upper limit. As for REM, since low radioactivity elements are easy to be handled when being mainly used, from this viewpoint, it is useful to use one or more selected from the group consisting of Sc, Y, La, Ce, Pr, Nd, Sm, Eu, Gd, Tb, Dy, Ho, Er, Tm, Yb and Lu. It is desirable to use light rare earth elements, especially La or Ce from the viewpoint of conspicuous exertion of the effect and price. However, there arises no trouble with mixing in of a trace of radioactive rare earth elements such as Th and U inevitably remaining, without being excluded, in a process to separate rare earth elements. Further, from the viewpoint of reduction in raw material cost, there can be used not-separated rare earth elements such as mish metal and didymium.

A free cutting alloy of the present invention constituted as stainless steel can contain one or more selected from the group consisting of Nb, V, Ta and Hf in each range of 0.01 to 0.5 mass %. Since Nb, V, Ta and Hf has an effect of forming carbo-nitrides to miniaturize crystalline particles of steel and increase toughness. Hence, the elements can add in each content up to 0.5 mass % and desirably contain 0.01 mass % or higher in the range.

A free cutting alloy of the present invention constituted as the above described stainless steel can contain the Wso value of which is less than 0.035 mass % when the following test is performed: an alloy test piece of said free cutting alloy is prepared so as to have the shape of rectangular prism in size of 15 mm in length, 25 mm in width and 3 mm in thickness with the entire surface being polished with No. 400 emery paper; a silver foil in size of 10 mm in length, 5 mm in width and 0.1 mm in thickness with a purity of 99.9 % or higher as a S getter; 0.5 cm³ of pure water are sealed in a vessel of an inner volume of 250 cm³ together with said test piece; the temperature in said vessel is raised to 85°C and said temperature is then kept there for 20 hr; and thereafter, the S content in mass % in said silver foil piece is analyzed, then S content obtained is defined as said Wso.

A (Ti, Zr) based compound being a feature of the present invention is formed and in the course of the formation, added S is included in the stainless steel as a constituting element of the (Ti, Zr) based compound which is more stable chemically than MnS or the like. And therefore, a S amount released into the air from the stainless steel decreases. Consequently, an out-gas resistivity of the stainless steel can also be improved by formation of the(Ti, Zr) based compound.

In this case, when the out-gas resistivity test is performed, a S component released from the test piece as a sulfur containing gas is forced to be absorbed in the silver foil as a getter and a sulfur content Wso in the silver foil is measured to quantitatively determine the out-gas resistivity of a material. A S content absorbed in the silver foil is defined using the Wso value and set to 0.035 mass % or lower in Wso. Stainless steel of the present invention controlled so as to be 0.035 mass % or lower in Wso is hard to cause sulfur contamination in the peripheral parts when exposed to the air since a S component released from the stainless steel into the air is very small and thereby the stainless steel can be preferably used as parts of industrial equipment requiring the out-gas resistivity.

While a factor determining out-gas resistivity of a material mainly is a composition of the material, it is desirable to fix S as carbo-sulfides of Ti and Zr for improvement on out-gas resistivity of the material. For the purpose, a S content is desirably determined such that a value of W_{S}/(W_{Ti} + 0.52W_{Zr}) is 0.45 or less, or alternatively a value of W_{S}/W_{C} is 0.4 or less and W_{S}/(W_{Ti}+ 0.52W_{Zr}) is 0.45 or less, wherein W_{S} and W_{C} denote a S content and a C content, respectively. With such a range of components adopted, a S content which is chemically in unstable condition can be limited and thereby, the out-gas resistivity of the matrix metal phase of stainless steel can be improved.

### Examples

The following experiments were performed in order to confirm the effects of the present invention. It should be appreciated that in the following description, test alloy relating to the present invention is referred to as inventive steel or inventive alloy, or as a selection inventive steel or a selection inventive alloy.

### Example 1 Ferrite containing stainless steel

The effects of a free cutting alloy constituted as ferrite containing stainless steel (a first selection inventive steel) were confirmed by the following experiment. First, 50 kg steel blocks with respective compositions in mass % shown in Table 1 were molten in a high frequency induction furnace and ingots prepared from the molten blocks were heated at a temperature in the range of from 1050 to 1100°C and the ingots were forged in a hot state into rods with a circular section of 20 mm diameter and the rods were further heated at 800°C for 1 hr, followed by air cooling (annealing) as a source for test pieces.

### Table 1

While main inclusions of an inventive steel of the present invention was (Ti,Zr)₄(S,Se)₂C₂, other inclusions such as (Ti,Zr)S and (Ti,Zr)S₃ are locally recognized in the matrix. Further, in a specimen No. 7 high in Mn content, (Mn, Cr)S is recognized, though in a trace amount. An identification method for inclusions was performed in the following way: A test piece in a proper amount was sampled from each of the rods. A metal matrix portion of the test piece was dissolved by electrolysis using a methanol solution including tetramethylammonium chloride and acetylaceton at 10 % as a electrolytic solution. The electrolytic solution after the electrolysis was subjected to filtration and compounds not dissolved in steel were extracted from the filtrate. The extract was dried and subjected to chemical analysis by an X-ray diffraction method with a diffractometer. A compound was identified based on peaks of a diffraction chart. A composition of a compound particle in the steel structure was separately analyzed by EPMA and a compound with a composition corresponding to a compound observed by X-ray diffraction was confirmed based on formation from two dimensional mapping results. Fig. 1 shows an X-ray diffraction chart of an inventive steel No. 5 by a diffractometer and Fig. 3 is an optical microphotograph of an inventive steel specimen No. 5. Further, specimens Nos. 1 to 14 in Table 1 are kinds of steel corresponding to the first selection inventive steel and specimens Nos. 15 to 28 are kinds of steel as comparative examples.

The following experiments were performed on the above described test pieces:

### 1) Hot workability test

Evaluation of hot workability was effected based on visual observation of whether or not defects such as cracks occur in hot forging. [○] indicates that substantially no defect occurred in hot forging, [×] indicates that large scale cracks were recognized in hot forging and △ indicates that small cracks occurred in hot forging.

### 2) Evaluation of machinability

Evaluation of machinability was collectively effected based on cutting resistance in machining, finished surface roughness and chip shapes. A cutting tool made of cermet was used to perform machining under a dry condition at a circumferential speed of 150 m/min, a depth of cutting per revolution of 0.1 mm and a feed rate per revolution of 0.05 mm. A cutting resistance in N as a unit was determined by measuring a cutting force generating in the machining. The finished surface roughness was measured by a method stipulated in JIS B 0601 and a value thereof was an arithmetic average roughness (in µm Ra) on a test piece surface after the machining. Moreover, chip shapes were visually observed and when friability was good, the result is indicated by [G] and when friability is bad and all chips are not separated but partly connected, the result is indicated by [B] and when evaluation of chip shapes is intermidiate of [G] and [B], the result is indicated by [I].

### 3)

### 4)Evaluation of out-gas resistivity

Evaluation of out-gas resistivity was performed by determining an amount of released S. To be concrete, test pieces in use each had the shape of a rectangular prism of 15 mm in length, 25 mm in width and 3 mm in thickness and the entire surface of each were polished with No. 400 emery paper. A test piece was placed in a sealed vessel having an inner volume of 250 cm³ together with a silver foil having a size of 10 mm in length, 5 mm in width and 0.1 mm in thickness and 0.5cm³ of pure water, and a temperature in the vessel was maintained at 85°C for 20 hr. A S content Wso in the silver foil after the process for the test was measured by a combustion type infrared absorbing analysis method.

### 4) Cold workability test

Evaluation of cold workability was performed by measuring a threshold compressive stain in a compression test on specimens Nos. 1 to 5 and 13. Test pieces for compression each had the shape of a cylinder of 15 mm in diameter and 22.5 mm in height and each piece was compressed by a 600 t oil hydraulic press to obtain a threshold compressive strain, wherein the threshold compressive strain is defined as In (H0/H) or a natural logarithm of H0/H, H0 being an initial height of the test piece and H being a threshold height which is a maximum height at which no cracking has occurred. First selection inventive alloys of the specimens Nos. 1 to 5 were confirmed to have high threshold compressive ratios almost equal to comparative steel specimen No. 15 and higher than comparative steel specimen No. 16 by about 20 %, and have a good cold workability as well.

### 5) Evaluation of corrosion resistivity

Evaluation of corrosion resistivity was performed by a salt spray test. Test pieces each were prepared so to have the shape of a cylinder of 10 mm in diameter and 50 mm in height. The entire surface of each test piece was polished with No. 400 emery paper and cleaned. A test piece was exposed to a fog atmosphere of 5 mass % NaCl aqueous solution at 35°C for 96 hr. Final evaluation was visually performed with the naked eye. As a result, the inventive steel of the present invention was confirmed to maintain good corrosion resistivity. The results are shown in Table 2.

### Table 2

It is found from Table 2 that first selection inventive steel of the present invention is comparable with conventional ferrite containing stainless steel in hot workability, cold workability and corrosion resistivity and moreover, is better in machinability than the conventional ferrite containing stainless steel. Further, it is found from Table 2 when comparing with comparative steel specimens Nos. 16 and 18 that the first selection inventive steel of the present invention is smaller in Wso and better in out-gas resistivity. The reason why kinds of steel of comparative alloy specimens Nos. 16 and 18 each have a high Wso is considered that since the steel of the kinds has neither Ti nor Zr, carbo-sulfide is hard to be formed, whereby a S amount in the matrix is excessively high. In comparative alloy specimen No. 18, hot workability is poor and therefore, evaluation of machinability was not performed.

## Claims

1. Free cutting alloy constituted as ferrite containing stainless steel containing:
2 mass % or lower, including zero, Ni; 12 to 35 mass % Cr; and 0.005 to 0.4 mass % C;
one or more of Ti and Zr such that W_{Ti} + 0.52 W_{Zr} = 0.03 to 3.5 mass %, wherein W_{Ti} and W_{Zr} denote respective contents in mass % of Ti and Zr;
and one or more of S and Se in the respective ranges of 0.01 to 1 mass % for S and 0.01 to 0.8 mass % for Se and
a (Ti,Zr) based compound containing one or more of Ti and Zr as a metal element component,
and wherein C is an indispensable element as a bonding component with the metal element component, and one or more of S, Se and Te is dispersed in a matrix metal phase; optionally further containing:
2 mass % or lower, including zero Si; 2 mass % or lower, including zero Mn; 2 mass % or lower, including zero Cu; 2 mass % or lower, including zero Co;
one or more of Mo and W in the respective ranges of 0.1 to 4 mass % for Mo and 0.1 to 3 mass % for W;
0.05 mass % or lower, including zero P; 0.03 mass % or lower, including zero O; 0.05 mass % or lower, including zero N;
one or more of Te, Bi and Pb in the respective ranges of 0.005 to 0.1 mass % for Te; 0.01 to 0.2 mass % for Bi; and 0.01 to 0.3 mass % for Pb;
one or more selected from the group consisting of Ca, Mg, B and REM (one or more of metal elements classified as Group 3A in the periodic table of elements) in the range of 0.0005 to 0.01 mass % for one element or as a total content of more than one elements combined;
one or more selected from the group consisting of Nb, V, Ta and Hf in each range of 0.01 to 0.5 mass %, the balance being Fe and inevitable impurities.

2. Free cutting alloy according to claim 1, wherein W_{S}/(W_{Ti}+0.52 W_{Zr}) is 0.45 or less, wherein W_{S}, W_{Ti} and W_{Zr} denote a S content, a Ti content and a Zr content, respectively.

3. Free cutting alloy according to any of claims 1 to 2, the Wso value representing the S amount released is less than 0.035 mass % when the following test is performed:
an alloy test piece of said free cutting alloy is prepared so as to have the shape of rectangular prism in size of 15 mm in length, 25 mm in width and 3 mm in thickness with the entire surface being polished with No. 400 emery paper;
a silver foil in size of 10 mm in length, 5 mm in width and 0.1 mm in thickness with a purity of 99.9 % or higher as a S getter;
0.5 cm³ of pure water are sealed in a vessel of an inner volume of 250 cm³ together with said test piece;
the temperature in said vessel is raised to 85°C and said temperature is then kept there for 20 hr;
and thereafter, the S content in mass % in said silver foil piece is analyzed, then S content obtained is defined as said Wso.

4. Free cutting alloy according to any one of claims 1 to 3, wherein a particle size of the (Ti, Zr) based compound as observed in the structure of a polished section of the alloy is in the range of 0.1 to 30 µm on the average, and further an area ratio of the compound in the structure is in the range of 1 to 20%.

## Patentansprüche

1. Automatenlegierung, welche als Ferrit-haltiger Edelstahl ausgebildet ist, enthaltend:
2 Massen-% oder weniger, einschließlich null, Ni; 12 bis 35 Massen-% Cr; und 0,005 bis 0,4 Massen-% C;
ein oder mehrere aus Ti und Zr, wobei W_{Ti} + 0,52 W_{Zr} = 0,03 bis 3,5 Massen-%, worin W_{Ti} und W_{Zr} die jeweiligen Anteile von Ti und Zr in Massen-% angeben, erfüllt ist;
und ein oder mehrere aus S und Se in den jeweiligen Bereichen von 0,01 bis 1 Massen-% für S und 0,01 bis 0,8 Massen-% für Se und
eine (Ti, Zr)-basierte Verbindung, welche ein oder mehrere von Ti und Zr als eine Metall-Element-Komponente enthält,
und worin C ein unabdingbares Element als Bindungskomponente mit der Metall-Element-Komponente darstellt, und wobei ein oder mehrere von S, Se und Te in einer Matrix-Metallphase dispergiert sind; wobei wahlweise weiterhin enthalten sind:
2 Massen-% oder weniger, einschließlich null, Si; 2 Massen-% oder weniger, einschließlich null, Mn; 2 Massen-% oder weniger, einschließlich null, Cu; 2 Massen-% oder weniger, einschließlich null, Co;
ein oder mehrere von Mo und W in den jeweiligen Bereichen von 0,1 bis 4 Massen-% für Mo und 0,1 bis 3 Massen-% für W;
0,05 Massen-% oder weniger, einschließlich null, P; 0,03 Massen-% oder weniger, einschließlich null, O; 0,05 Massen-% oder weniger, einschließlich null, N;
ein oder mehrere aus Te, Bi und Pb in den jeweiligen Bereichen von 0,005 bis 0,1 Massen-% für Te; 0,01 bis 0,2 Massen-% für Bi; und 0,01 bis 0,3 Massen-% für Pb;
ein oder mehrere, ausgewählt aus der Gruppe, bestehend aus Ca, Mg, B und REM (ein oder mehrere der als Gruppe 3A in dem Periodensystem der Elemente klassifizierten Metallelemente) in dem Bereich von 0,0005 bis 0,01 Massen-% für ein Element oder als Gesamtgehalt von mehr als einem Element in Kombination;
ein oder mehrere, ausgewählt aus der Gruppe, bestehend aus Nb, V, Ta und Hf in dem jeweiligen Bereich von 0,01 bis 0,5 Massen-%, wobei der Rest Fe und unvermeidbare Verunreinigungen sind.

2. Automatenlegierung nach Anspruch 1, worin W_{S}/(W_{Ti}+0,52 W_{Zr}) 0,45 oder weniger beträgt, worin W_{S}, W_{Ti} und W_{Zr} jeweils einen S-Gehalt, einen Ti-Gehalt und einen Zr-Gehalt bedeuten.

3. Automatenlegierung nach einem der Ansprüche 1 bis 2, wobei der Wso-Wert, welcher den freigesetzten S-Gehalt darstellt, geringer als 0,035 Massen-% ist, sofern der folgende Test durchgeführt wird:
ein Legierungsteststück der Automatenlegierung wird derartig hergestellt, dass es die Form eines rechteckigen Prismas der Größe von 15 mm in der Länge, 25 mm in der Breite und 3 mm in der Dicke aufweist, wobei die Gesamtoberfläche mit einem Schmirgelpapier der Nr. 400 poliert wurde;
eine Silberfolie der Größe von 10 mm in der Länge, 5 mm in der Breite und 0,1 mm in der Dicke mit einer Reinheit von 99,9% oder mehr als S-Getter;
0,5 cm³ reines Wasser werden in ein Gefäß mit einem Innenvolumen von 250 cm³ zusammen mit dem Teststück versiegelt;
die Temperatur in dem Gefäß wird auf 85°C erhöht, und die Temperatur wird anschließend 20 Stunden lang dort gehalten;
und anschließend wird der S-Gehalt in Massenprozent in der Silberfolie analysiert, wobei der erhaltene S-Gehalt als der Wso definiert ist.

4. Automatenlegierung nach einem der Ansprüche 1 bis 3, worin die Teilchengröße der (Ti, Zr)-basierten Verbindung, wie sie in der Struktur eines polierten Abschnitts in der Legierung beobachtet wird, in dem Bereich von durchschnittlich 0,1 bis 30 µm liegt und wobei weiterhin ein Flächenverhältnis der Verbindung in der Struktur in dem Bereich von 1 bis 20% liegt.

## Revendications

1. Alliage de décolletage constitué de ferrite contenant un acier inoxydable comprenant :
2 % en masse ou moins, zéro inclus, de Ni ; de 12 à 35 % en masse de Cr ; et de 0,005 à 0,4 % en masse de C ;
un ou plusieurs éléments choisis parmi Ti et Zr de sorte que W_{Ti} + 0,52W_{Zr} = 0,03 à 3,5 % en masse, dans W_{Ti} et W_{Zr} représentant respectivement les teneurs en % en masse de Ti et Zr ;
et un ou plusieurs éléments choisis parmi S et Se dans les plages respectives de 0,01 à 1 % en masse pour S et de 0,01 à 0,8 % en masse pour Se ; et
un composé de (Ti,Zr) contenant un ou plusieurs éléments choisis parmi Ti et Zr en tant que composant de type élément de métal ;
et dans lequel C est un élément indispensable en tant que composant de liaison avec le composant de type élément de métal, et un ou plusieurs éléments choisis parmi S, Se et Te sont dispersés dans une phase métallique formant matrice ; contenant en outre éventuellement :
2 % en masse ou moins, zéro inclus, de Si ; 2 % en masse ou moins, zéro inclus, de Mn ; 2 % en masse ou moins, zéro inclus, de Cu ; 2 % en masse ou moins, zéro inclus, de Co ;
un ou plusieurs éléments choisis parmi Mo et W dans les plages respectives de 0,1 à 4 % en masse pour Mo et de 0,1 à 3 % en masse pour W ;
0,05 % en masse ou moins, zéro inclus, de P ; 0,03 % en masse ou moins, zéro inclus, de O ; 0,05 % en masse ou moins, zéro inclus, de N ;
un ou plusieurs éléments choisis parmi Te, Bi et Pb dans les plages respectives de 0,005 à 0,1 % en masse pour Te ; de 0,01 à 0,2 % en masse pour Bi ; et de 0,01 à 0,3 % en masse pour Pb ;
un ou plusieurs éléments choisis parmi le groupe consistant en Ca, Mg, B et les éléments de métal de terre rare (REM) (un ou plusieurs des éléments de métal classés en tant que groupe 3A dans le tableau périodique des éléments) dans la plage de 0,0005 à 0,01 % en masse pour un élément ou en tant que teneur totale de plus d'un élément associé ;
un ou plusieurs éléments choisis parmi le groupe consistant en Nb, V, Ta et Hf chacun dans la plage de 0,01 à 0,5 % en masse, le reste consistant en Fe et en impuretés inévitables.

2. Alliage de décolletage selon la revendication 1, dans lequel W_{S}/(W_{Ti} + 0,52W_{Zr}) est de 0,45 ou moins, et dans lequel Ws, W_{Ti} et W_{Zr} représentent respectivement la teneur en S, la teneur en Ti et la teneur en Zr.

3. Alliage de décolletage selon l'une quelconque des revendications 1 et 2, la valeur W_{SO} représentant la quantité de S libéré, est inférieure à 0,0 35 % en masse lorsque l'essai suivant est effectué :
une éprouvette d'alliage du dit alliage de décolletage est préparée de façon à avoir la forme d'un prisme rectangulaire d'une taille de 15 mm de longueur, de 25 mm de largeur et de 3 mm d'épaisseur dont la totalité de la surface est polie avec du papier d'émeri N° 400 ;
on prévoit une feuille d'argent d'une taille de 10 mm de longueur, de 5 mm de largeur et de 0,1 mm d'épaisseur, ayant une pureté de 99,9 % ou plus, en tant que piège pour S ;
on enferme hermétiquement 0,5 cm³ d'eau pure dans un récipient d'un volume intérieur de 250 cm³ ensemble avec ladite éprouvette ;
la température du dit récipient est accrue jusqu'à 85 °C, et ladite température est ensuite maintenue pendant 20 h ; et
la teneur en S exprimée en % en masse dans ladite pièce de feuille d'argent, est ensuite analysée, la teneur en S obtenue étant alors définie comme étant ladite valeur W_{SO}.

4. Alliage de décolletage selon l'une quelconque des revendications 1 à 3, dans lequel la taille particulaire du composé de (Ti,Zr) observé dans la structure d'une section polie de l'alliage, est dans la plage de 0,1 à 30 µm en moyenne, et dans lequel le taux de surface du composé dans la structure est dans la plage de 1 à 20 %.
